

## UNITED STATES PATENT OFFICE

2,229,858

## LUBRICANT MANUFACTURE

Elliott B. McConnell, Shaker Heights, Ohio, assignor to The Standard Oil Company, Cleveland, Ohio, a corporation of Ohio

No Drawing. Application October 22, 1938,  
Serial No. 236,553

4 Claims. (Cl. 252—50)

In the operation of internal combustion engines, the lubricating oil is exposed to extremely drastic conditions, and changes occur in the oil and degradation products tend to be formed rather profusely. A particular difficulty lies in the fact that the substances formed are of adhesive character and prone to stick the piston rings, preventing proper sealing, and interfering with normal operation. I have found that certain compounds afford a surprisingly effective lubricant for heavy duty operations. The action is not explainable merely as of anti-oxidant character, as sometimes ascribed to lubricating oils; as it is effective also in absence of oxygen, and considering the difference in what degradation products are formed, in comparison with those in a plain mineral oil of the same viscosity, it may be concluded that the lighter bodied, lighter colored resinous material formed is a relatively lower product of polymerization, and an important practical effect is that its nature is unctuous and oily instead of adhesive and sticky as with mineral oil per se.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

A mineral lubricating oil stock of desired viscosity is employed as the base of the present lubricant, and with it is incorporated a cyclohexyl compound which is of amine type. For instance, monocyclohexyl amine, dicyclohexyl amine, tricyclohexyl amine. The amount of the cyclohexyl compound need not be large. It need not exceed 5 per cent in general, and amounts as low as 0.01 per cent are sufficient in many instances. The lubricating oil stock may be for example an oil of 75 to 150 sec. Saybolt viscosity at 210° F., as derived from any suitable petro-

leum, as Pennsylvania, Mid-Continent, etc. The miscibility of these cyclohexyl compounds is such that they readily incorporate into the oil at generally ordinary temperature. Any special refining treatment of the oil which may have been desired, should have been carried out prior to this compounding.

As an example: A Mid-Continent lubricating stock of S. A. E. 30, in amount 99.5 per cent, and dicyclohexyl amine in amount 0.5 per cent are thoroughly incorporated together. This composition applied as a crankcase lubricant in an internal combustion engine shows remarkable ability to stand up under long continued runs continuously, without interruption from ring sticking, and the resinous material which occurs is peculiar in being greasy instead of sticky, and it is not easily decomposed by temperatures around 400—500° F., but retains its smooth unctuous character.

Similarly, monocyclohexyl amine and tricyclohexyl amine may be substituted as in the above, as may be desired in any instance.

Other modes of applying the principle of the invention may be employed, change being made as regards the details described, provided the features stated in any of the following claims, or the equivalent of such, be employed.

I therefore particularly point out and distinctly claim as my invention:

1. A lubricant, comprising a mineral oil of lubricating viscosity and a small amount of a cyclohexyl amine.
2. A lubricant, comprising a mineral oil of lubricating viscosity and a small amount of dicyclohexyl amine.
3. A lubricant, comprising a mineral oil of lubricating viscosity and a small amount of tricyclohexyl amine.
4. A lubricant, comprising a mineral oil of lubricating viscosity and a small amount of monocyclohexyl amine.

ELLIOTT B. McCONNELL.